

1,016,560.

F. GIOLITTI.  
ARMOR PLATE AND OTHER STEEL ARTICLE.  
APPLICATION FILED OCT. 10, 1907.

Patented Feb. 6, 1912.



*Witnesses:*

L. B. Badeau.  
H. D. Penney

*Inventor:*

Federico Giolitti.  
By his Attorney, F. W. Richards

# UNITED STATES PATENT OFFICE.

FEDERICO GIOLITTI, OF ROME, ITALY, ASSIGNEE TO SOCIETA ANONIMA ITALIANO GIO ANSALDO ARMSTRONG & CO., OF GENOA, ITALY, A COMPANY INCORPORATED IN ITALY.

## ARMOR-PLATE AND OTHER STEEL ARTICLE.

1,016,560.

Specification of Letters Patent.

Patented Feb. 6, 1912.

Original application filed September 8, 1906, Serial No. 333,408. Divided and this application filed October 10, 1907. Serial No. 396,864.

To all whom it may concern:

Be it known that I, FEDERICO GIOLITTI, a subject of the King of Italy, residing in Rome, Italy, have invented certain new and 5 useful Improvements in Armor-Plates and other Steel Articles, of which the following is a specification.

This application is a division out of an application filed in the United States Patent Office Sept. 6, 1906, Serial No. 333,408.

This invention relates to armor plates or other objects made of steel, composed of either superficial or deep successive zones in steels of different composition, not only as 15 regards the proportion of carbon contained but also as regards the presence in some of them of foreign metals and as regards the proportions in which these metals enter into the composition. This latter varies gradually in passing from one zone to another.

The accompanying drawing illustrates diagrammatically a steel plate after treatment according to the present invention.

The result in question is obtained by sub- 25 mitting the mass of homogeneous steel (either ordinary carbon steel or a special ternary, quaternary or like steel) to the action of suitable granular mixtures containing the metal it is desired to introduce into 30 the steel, such for instance, as chromium, nickel, tungsten, molybdenum, manganese, vanadium and sometimes silicon and uranium in a free state or in a state readily dissociated under certain conditions, which, 35 as hereinafter set forth, varies from one preparation to the other as well as from one phase to the other of the same preparation. These granular mixtures are strongly pressed against one or both surfaces of the 40 plate or other article that is treated.

For each given composition of the homogeneous steel which forms the mass under manipulation, as well as for one or more of the given metals contained in the mixture 45 employed, there exists a determined range of temperature, which depends strictly on the range of the critical points of the homogeneous steel itself, and on the nature of the metals employed. It is in this range that 50 occurs the diffusion of the metal or metals contained in the mixture pressed against the surfaces of the mass of steel, toward the interior of the mass. The range of temperature referred to which is the most suitable

for obtaining the diffusion in question, is 55 comprised between the temperature of the first critical point of the steel employed and a temperature below its point of fusion. The depth to which the metal contained in the granular mixture extends into the homogeneous mass of steel submitted to such an operation, depends primarily on the duration of the operation; but even by considerably prolonging this duration, a very deep 60 or gradual diffusion would not be obtained 65 in the greater number of cases if the temperature were always maintained constant from the beginning of the operation until the end.

The constancy of the temperature—a condition which would be very useful if a certain concentration as regards the foreign metal introduced had not been surpassed, and if a great homogeneousness of concentration for a given zone of the plate had to 70 be obtained, prevents a very definite given limit of concentration being surpassed, because if this latter is increased there is produced a displacement of the critical points and consequently of the interval of temperature in which the diffusion can be effected. It results that at a certain moment the temperature maintained constant is no longer 75 comprised in this interval and consequently 80 the passage of the metal of the mixture to 85 the mass under treatment is no longer effected and the diffusion is effected only at the interior of the mass until the concentration is suitably lowered owing to the interior diffusion referred to. It will then generally be advisable to suitably alternate the 90 reduction and the increases of temperature in limits which can easily be determined for each case and which generally ought to determine the critical points.

The product of the treatment referred to above will consist of a heterogeneous mass of steel, the composition of which varies in the various zones or layers according to the composition of the micro-construction of the 100 homogeneous steel at the beginning, the composition of the granular mixture employed, and the fixed or variable conditions of temperature in which the operation is effected. For example, if the process is begun with an ordinary homogeneous carbon steel ingot and a granular mass containing only one metal is used for the treatment, and

pressed against only one face of the ingot, the result will be (beginning with the surface which has been submitted to the operation) a body formed of a ternary steel in which the proportion of the characteristic steel forming metal decreases toward the interior of the body, until at a certain depth, this proportion is reduced to zero. From this point the ingot will still be formed of the same original carbon steel which may have (as well as the ternary zone) the same initial proportion of carbon, or a different proportion according as the granular mass did or did not contain active substances or was more or less rich in carbon or metallic oxid. As example a steel carbon plate (0.1 to 0.2 per cent. of carbon) may be taken, maintained in contact with a mixture of wolframic acid and of substances suitably "carbonaceous", or nitrogenous, compressed against one of its surfaces at a temperature near that of fusion. As an example of such nitrogenous substances may be mentioned: charcoal 50%, bone black 20%, carbonate of barium 25%, and ferrocyanid of potassium 5%. In this case the preceding operation must be followed by a superficial de-carbonization, obtained by means of heating in contact with mixtures of metallic oxids. On the contrary, if a start is made with a ternary homogeneous steel ingot (for example, a chrome steel with two to four per cent. of chromium) the final product will have a structure similar to that of the former ingot, but the layer of ternary steel would be substituted by a layer of quaternary steel, while the rest of the body would still be ternary steel. In the case just mentioned, by employing a mixture of the preceding case, the quaternary layer will consist of chrome steel and wolfram steel. The procedure is followed in a similar manner for the more complex steels.

Similar considerations will apply in the case where the treatment by diffusion is effected on two surfaces or on all the surface of the steel objects, in one, two, or more times; these operations alternating with thermic treatment (temperings and the like) or suitable mechanical operations which may vary for each case according to the nature of the steel employed and of the steel desired to be obtained. The operation just referred to may be applied directly to the mass of homogeneous steel as cast, or to the mass when brought to the desired shape by the mechanical manipulations, such as hammering, rolling, pressing and the like. In every instance, however, it would almost always be necessary to follow the chemical treatment described by a suitable thermic treatment. But it is in the temper of the metallic bodies where the greatest advantages of this method of manufacture and the superiority of the bodies produced in this manner,

are evident as compared with those obtained by other methods. As a matter of fact, by employing this method, any desired composition for the various zones of the body of steel, can be obtained, and consequently various parts of the object may be given the most suitable composition by means of a homogeneous tempering applied to the whole whereby each part acquires physical, chemical or mechanical properties (such as magnetic properties, resistance to chemical agents, hardness, plasticity, elasticity and the like) the most suitable for the purposes for which the bodies are to be employed. By this method, armor plates for example, can be obtained which, after one or more homogeneous temperings effected under the desired conditions of temperature and the like, possess mechanical properties (hardness, tenacity, and the like) differing in the various layers so that they can be most suitably adapted to the most varied uses.

Let us suppose for example to have to do with a special nickel steel showing the following composition: Nickel 2.20%, carbon 0.10%, manganese 0.42%, silicon 0.30%, sulfur 0.04% phosphorus 0.02%, and that it be intended to obtain a zone of 3 mm. thickness, in which the percentage of carbon should vary from 0.9% (on the outer face) down to 0.4% at 3 mm. depth, while the percentage of manganese, namely of the metal to be introduced by diffusion according to the present invention should vary between 3% (on the outer face) and 0.7% at 3 mm. depth. In order to obtain this result it will be sufficient to heat the steel piece in contact with a granular mixture consisting of three parts of charcoal, one of finely pulverized manganese dioxid and one of barium carbonate. A temperature of 1150 degrees C. is to be kept up during about half an hour; whereupon the same is to be allowed to gradually drop down to 700 degrees C. at the end of three hours. In making these statements, as to the duration of the heating, it has been assumed that the time begins to run since the full heat has been laid on the steel pieces; the additional time necessary for reaching the aforesaid temperatures as well for cooling after each treatment, of course depends upon the size of the pieces and the arrangement of the heating furnaces.

Having described my invention I claim:

1. A steel plate or other article having on one or more surfaces a zone of considerable thickness throughout which is diffused a characteristic metallic steel component not contained in the other part of the article, the said metallic component being graded from a maximum inwardly to a minimum, such zone having a less proportion of carbon than in the other portion of the article.

2. A ternary steel plate or other article having on one or more surfaces a quaternary zone of considerable thickness throughout which is diffused a characteristic metallic 5 steel component not contained in the other part of the article, the said metallic component being graded from a maximum inwardly to a minimum, such zone having a

less proportion of carbon than in the other portion of the article.

Signed at Nos. 9-15 Murray street, New York, N. Y., this first day of October, 1907.

FEDERICO GIOLITTI.

Witnesses:

WILLIAM H. REID,

FRED. J. DOLE.